

## UNITED STATES PATENT OFFICE

2,015,703

## PROCESS FOR PRODUCING HIGHLY REFINED ANTIDETONATION MOTOR FUEL

Norman Frank Black and Joshua A. Tilton,  
Baton Rouge, La., assignors to Standard-I.G.  
CompanyNo Drawing. Application May 14, 1931,  
Serial No. 537,498

## 2 Claims. (Cl. 196—40)

This invention relates to the preparation of highly refined motor fuel and more specifically comprises an improved method of finishing motor fuel which has been prepared by the hydrogenation of higher boiling hydrocarbons.

Our improved process will be fully understood from the following description.

Hydrocarbon oils, higher boiling than are suitable for motor fuel, are heated to a temperature in excess of 350° F. and are forced into a reaction chamber which is maintained under pressure in excess of 20 atmospheres, preferably 100 or 200 atmospheres or higher, and at temperatures between about 900 and 1100° F.

Hydrogen or a gas rich in free hydrogen is also forced into the reaction chamber and is preferably added in admixture with the oil. In the reaction chamber the higher boiling hydrocarbons are subjected to hydrocyclification and are substantially completely converted to hydrocarbons boiling below about 450° F. Such hydrocarbons as are not converted on one passage through the reaction chamber may be continuously recycled.

The reaction chamber preferably contains a catalytic material which greatly increases the rate of hydrocyclification. The oxides or sulfides of metals of the II, IV, and VI groups of the periodic system are suitable catalytic materials for this purpose, among which the oxides or sulfides of chromium, tungsten and molybdenum, preferably in combination with the oxides of zinc or magnesium, are especially satisfactory. All of these materials are immune to sulfur poisoning.

Vapors flowing out of the reaction chamber are cooled, preferably by interchange of heat with cold feed material, and by further cooling if necessary and uncondensed gases are separated from the liquid products. The uncondensed gases which contain a substantial quantity of unused hydrogen may be scrubbed with oil, acid or alkali or any combinations of these to rid them of hydrogen sulfide, ammonia, hydrocarbon gases and other impurities and the purified gas may be recirculated to the reaction chamber.

The liquid products may then be passed into a fractionating tower wherein they may be separated into two fractions, one containing hydrocarbons boiling below about 450°, 400°, or

350° F. and the other containing hydrocarbons of higher boiling point range. The latter fraction may be recirculated to the reaction chamber for further treatment.

The lighter fraction is suitable for motor fuel and is characterized by exceptionally low sulfur and gum content and has marked anti-detonation characteristics. We have found that it may be still more highly refined and at the same time have its anti-detonation properties even further increased by subjecting it to the following finishing treatment:

The hydrogenated oil is treated with sulfuric acid at relatively low temperatures. Between about 2 and 5 pounds of 98% sulfuric acid per 15 barrel is preferable and temperature should be maintained below about 80° F. and preferably about 35° F. A greater amount of acid or a higher temperature of treatment may be used, but the results are not as good as those obtained under the preferred conditions. Following the acid treatment the excess acid is neutralized by the addition of an alkali such as caustic soda or lye and the mixture is then subjected to fire and steam distillation. The maximum temperature 25 to which the oil is heated during the distillation is preferably not above about 300° F. The distillation may be carried out in the presence of clay, such as for example Atapulgus clay. About 4 pounds of 200 mesh clay per barrel of oil 30 is sufficient but more or less than this may be used with satisfactory results.

As an example of this method of finishing hydrogenated motor fuel, a 400° F. E. P. distillate is separated from the product of hydrocyclification of a Mid-Continent gas oil of boiling range 450 to 600° F. This distillate has the following characteristics:

|                       |           |    |
|-----------------------|-----------|----|
| Gravity A. P. I.      | 51.6°     | 40 |
| Octane number         | 69.0      |    |
| Gum (porcelain dish)  | 113.1 mg. |    |
| Color (Robinson)      | +12       |    |
| Initial boiling point | 134° F.   |    |
| Final boiling point   | 403° F.   | 45 |
| Sulfur                | .005%     |    |

It is treated with 2 pounds of 98% sulfuric acid per barrel of oil at a temperature of 80° F. The acid is neutralized by the addition of caustic alkali and the mixture is steam distilled at a 50

maximum oil temperature of 300° F. The finished distillate thus obtained has the following characteristics:

|    |                       |          |
|----|-----------------------|----------|
| 5  | Gravity A. P. I.      | 53.0°    |
|    | Octane number         | 74.8     |
|    | Gum (porcelain dish)  | 12.4 mg. |
|    | Color (Robinson)      | +25      |
| 10 | Initial boiling point | 120° F.  |
|    | Final boiling point   | 391° F.  |
|    | Sulfur                | .04%     |

The octane number is the percent of iso-octane which must be added to normal heptane to give a mixture having the same anti-detonation value 15 as the motor fuel. Thus the higher the octane number, the greater is the anti-detonation value of the fuel.

It will be observed that the color and gum have been markedly improved and that the octane 20 number has been increased from 69.0 to 74.8 which is a substantial improvement.

To show the effect of the temperature at which the acid treatment is carried out, a 300° F. E. P. distillate obtained from the hydrocyclification 25 of the same Mid-Continent gas oil is treated at 35° F. and 80° F. respectively with the following results:

| 30 | Untreated             | Treated with                                                 | Treated with                                   |
|----|-----------------------|--------------------------------------------------------------|------------------------------------------------|
|    |                       | 5 lbs. 98% H <sub>2</sub> SO <sub>4</sub> /bbl. temp. 35° F. | 5 lbs. 98% sulfuric acid per bbl. temp. 80° F. |
| 35 | Gravity A. P. I.      | 59.9                                                         | 59.7                                           |
|    | Octane number         | 73.8                                                         | 78.5                                           |
|    | Gum (porcelain dish)  | 2.4                                                          | 2.0                                            |
|    | Color (Robinson)      | +12                                                          | +25                                            |
|    | Initial boiling point | 110                                                          | 110                                            |
|    | Final boiling point   | 288                                                          | 290                                            |

It will be observed that when the acid treatment is carried out at 35° F. the increase in octane number is greater than it is when the acid treatment is at 80° F.

As a second example a 432° F. E. P. gasoline separated from the product of hydrocyclification of the heavy naphtha bottoms of Coastal crude is treated with 2 pounds 98% sulfuric acid per barrel at a temperature of 80° F. and fire and steam distilled. The characteristics of the oil before and after treatment are as follows:

| 50 |                       | Untreated | Treated  |
|----|-----------------------|-----------|----------|
|    |                       |           |          |
| 55 | Gravity A. P. I.      | 38.1      | 38.3     |
|    | Octane number         | 83.6      | 85.6     |
|    | Gum (porcelain dish)  | 48.4 mg.  | 10.0 mg. |
|    | Color (Robinson)      | +5        | +25      |
|    | Initial boiling point | 129° F.   | 138° F.  |
|    | Final boiling point   | 432° F.   | 434° F.  |

It will be observed that with this motor fuel also which was obtained by the hydrocyclification of an entirely different type of gas oil than the one in the previous example, the color and gum have been markedly improved and the octane number has also been substantially increased, from 83.6 to 85.6.

We are aware that the acid treatment of straight-run or cracked gasoline generally causes a decrease in the anti-detonation value of the motor fuel, and while we are not able to state the exact reasons for the opposite behavior of hydrogenated gasolines in this respect, we have found that the acid treatment of the hydrogenated motor fuels carried out in the manner described consistently results in an increase in the anti-detonation value. This effect is particularly noticeable with motor fuels produced in a vapor phase hydrogenation or hydrocyclification process which is intended to denote a process of destructive hydrocarbon carried out at temperatures above 900° F. and with a pressure of hydrogen adapted to produce largely unsaturated products on the one hand, and to prevent coke and tar formation on the other. In most cases the hydrogenated motor fuels are sufficiently refined by the hydrogen treatment in respect to color and gum forming properties, and the additional acid treatment is not usually necessary for finishing purposes, or at most is only necessary to a more limited extent than with the cracked gasolines. The fact however, that the acid treatment also causes a substantial increase in the anti-detonation value of the hydrogenated motor fuel makes such treatment especially desirable.

This invention is not limited by any theory of the mechanism of the reactions nor by any examples given merely for purposes of illustration, but only by the following claims in which we wish to claim all novelty inherent in the invention.

We claim:

1. An improved process for finishing naphthas of the type of gasoline and prepared by destructive hydrogenation of high boiling hydrocarbons which comprises treating the naphtha with sulfuric acid of substantially 98% strength at a temperature from about 35° to 80° F. whereby the naphtha is improved with respect to color and gum content and its anti-detonation value remains undiminished.

2. The process according to claim 1 in which 2 to 5 pounds of sulfuric acid per barrel of oil is used for treating.

NORMAN F. BLACK.  
J. ATWOOD TILTON.